

## UNITED STATES PATENT OFFICE

2,096,146

CELLULOSIC STRUCTURES AND METHOD  
OF PREPARING SAME

Fenton H. Swezey, Waynesboro, Va., assignor, by  
mesne assignments, to E. I. du Pont de Nemours & Company, Wilmington, Del., a corporation of Delaware

No Drawing. Application June 11, 1935,  
Serial No. 26,093

6 Claims. (Cl. 18—54)

This invention relates to non-fibrous cellulosic pellicles, threads, bands, tubes and the like, and more particularly relates to colored pellicles, threads, bands, tubes and the like produced from cellulose esters, and the method of preparing such colored structures.

Great difficulty has been experienced in the coloring of cellulose esters, for example, cellulose acetate, so as to obtain a colored pellicle, thread or fabric in which the color or dye is fast to light and to an alkaline scouring boil-off operation. Since the production of cellulose acetate yarn on a commercial scale, it has been found necessary to develop new dyes and/or methods of dyeing whereby to produce a desirable product, inasmuch as previously known dyes were found to be inefficient and in a great many cases inoperative for the dyeing of cellulose acetate.

These newly developed dyes are in some cases quite expensive or involve expensive methods of applying them to the yarn or fabric. Furthermore, the colors available in these new dyes are somewhat limited in comparison to the available colors in previously known dyestuffs, the use of which was found to be inexpedient for dyeing cellulose acetate materials.

By using previously known dyestuffs through modified methods of application fair results were obtained in some cases but such modified procedures were often expensive and time-consuming, and often depended upon the use of an expensive auxiliary dyeing medium. Furthermore, both the newly developed dyes and modified methods of applying previously known dyes generally involve a poor exhaustion of the dye from the dye baths.

Acid dyes and particularly water-soluble acid dyes are generally known to possess very little or no affinity for cellulose esters, such as cellulose acetate, and in fact advantage has been taken of the relatively small affinity of acid dyes to cellulose acetate to impart fugitive tints to acetate thread. In case of a few acid dyes a more or less permanent coloration results on the thread, if a solvent for cellulose derivative is present in the thread, but even these dyes cannot be applied in a manner to give a uniformly dyed thread, and generally they will not withstand boiling with water containing a small amount of sodium carbonate.

The surprising discovery has now been made that cellulose esters, such as cellulose acetate, can be successfully dyed with water-soluble acid dyes by incorporating a solution or suspension of the said acid dyes in a cellulose ester solution prior

to the formation of pellicles or filaments therefrom. The colored structures formed from such colored solutions of cellulose acetate or the like are found to be fast to light and comparatively fast to alkaline scouring boil-off solutions.

Although it is generally known to incorporate dyes in solutions of cellulose acetate, such previously known processes are limited to the use of insoluble colored pigments, to compounds which will form insoluble dyes upon subsequent treatment, and to water-insoluble dyes.

It is therefore an object of this invention to produce colored films, filaments and fabrics of cellulose esters, such as cellulose acetate, dyed with water-soluble acid dyes which are substantially fast to light and scouring boil-off operations.

It is a further object of this invention to produce films, filaments and fabrics of cellulose esters, such as cellulose acetate, having water-soluble acid dyes incorporated throughout the body thereof.

It is another object of this invention to provide a method of producing water-soluble acid dye-stuff colored films, fabrics and filaments of cellulose esters, such as cellulose acetate, which colors are fast to light and scouring boil-off operations.

Other objects of the invention will appear hereinafter.

The objects of the invention can be accomplished in general by dissolving or suspending water-soluble acid dyestuffs in hot or cold water or other suitable liquid medium, mixing a quantity of the dye solution or suspension with a quantity of a solution of a cellulose ester to obtain a uniform dispersion and spinning or casting the colored cellulose ester into the form of a filament or film.

By the term "acid dyes" as used throughout the specification and claims is meant not only those members of the triphenylmethane group generally classified as acid dyes, but also those dyes which contain one or more sulfonic acid groups in the form of sodium, potassium, calcium or ammonium salts or which contain phenol groups associated with nitro groups.

The present invention has particular utility and is described with specific reference to the dyeing of cellulose acetate structures. It is nevertheless to be understood that it is not to be limited thereto but that the invention is generally applicable to the production of colored films and filaments of cellulose esters, such as cellulose formate, cellulose propionate, cellulose butyrate, cellulose phthalate, and mixed cellulose esters, such as cellulose acetate formate, cellulose ace-

tate-propionate, cellulose propionate-butyrate and the like.

A water-soluble acid dye, such as Pontacyl Carmine 2—G, (Rowe Color Index No. 31), Pontacyl Brilliant Blue A, (Rowe Color Index No. 714), Pontacyl Black BX, (Rowe Color Index No. 246), Pontacyl Fast Red AS, (Rowe Color Index No. 176), Pontacyl Light Yellow 3—G (Rowe Color Index No. 636), or Pontacyl Fast Black BBO, (Rowe Color Index No. 307), is dissolved in hot or cold water or other appropriate liquid medium to form a solution, suspension or paste of suitable consistency and depending upon the shade desired. The resulting dye solution or paste is then thoroughly mixed with a suitable quantity of a solution of cellulose acetate, for example, a solution of cellulose acetate in acetone. The solution of cellulose acetate may, if desired, contain natural or synthetic resins, plasticizers, softeners or similar compounds such as may be added to produce cellulose acetate structures having special characteristics. The mixing of the solution of cellulose acetate and the dye solution may be carried out in any suitable manner by reason of the fact that the solutions can be easily and quickly brought to a homogeneous mixture. The resultant homogeneously colored mixture is then spun or cast into filaments or films by any of the conventional dry or wet methods.

The acid dye may, if desired, be added in its solid form to a solution of a cellulose ester already containing a solvent in suitable proportions, and dispersed by suitable homogenization methods.

Among the liquid mediums which may be substituted for water to form solutions or suspensions with the acid dyes may be mentioned acetone, mono-, di-, or polyhydric alcohols, esters, aniline, nitrobenzene, ethylene chloride, mono-, di-, or tri-alkylol amines, or mixtures of two or more thereof.

The depth of color imparted to the materials may be exactly and easily regulated by varying the amount of dye added to the cellulose acetate solution. Any color or shade known in the present art may thus be obtained in accordance with this invention. Furthermore, acid dyestuffs may be blended with vat dyes, basic dyes, and other classes of dyes, by proper care of selection, such as is well known in the art, and mixed with a solvent and a cellulose acetate solution to obtain very satisfactory results.

The quantity of water or other solvent or liquid medium in which the water-soluble acid dyestuff is dissolved or suspended should not exceed 20% by weight of the dyed cellulose ester solution or suspension when a thread or film of good physical characteristics is desired, and preferably the quantity of said water or other liquid medium is kept below 10% or even 5% by weight of the dyed cellulose ester solution.

If it is desired to obtain a delustered or opaqued colored film or filament, inorganic pigments, such as titanium oxide, barium oxide, zinc oxide or antimony white, or organic delusterants, can be incorporated in the dyed cellulose ester solution in the usual manner.

Threads dyed in accordance with this invention can in addition be temporarily tinted with fugitive dyes for purposes of identification and which may later be removed, if desired, without affecting the permanent colors imparted thereto.

In order to more clearly set forth the process and resultant product of the present invention, the following illustrative examples are given, it

being understood that the invention is not to be limited thereto in any way.

#### Example I

A quantity of Pontacyl Carmine 2—G (Color Index No. 31) is dissolved in water at room temperature and the resulting solution is diluted to a concentration of 2 grams per liter. A suitable quantity, for example, 8 cc. of the dye solution is added to 1000 grams of a 26% solution of cellulose acetate in acetone. The substances are agitated to form a uniformly homogeneous mixture in any desirable manner. A film or thread which is cast or spun from the mixture is dyed a pink color which is of excellent fastness to light and to an alkaline scouring boil-off operation.

#### Example II

A 1% aqueous solution of Pontacyl Brilliant Blue A (Color Index No. 714) is added to a 25% solution of cellulose acetate in acetone, in the proportion of about 30 cc. dye solution to 1000 grams acetate solution. The cellulose acetate solution contains sufficient finely divided delusterant, such as titanium oxide, to produce a dull thread. The components are agitated to form a uniform mixture, and the mixture is spun or cast into a thread or film which is colored a light blue and which is of excellent fastness to light and to an alkaline scouring boil-off operation.

#### Example III

A 9% paste is made of Pontacyl Black BX (Color Index No. 246) and hot water. This paste is added with stirring to a 22% solution of cellulose acetate in acetone in the proportion of about 58 grams paste to 1000 grams acetate solution.

The components are agitated to form a homogeneous mixture which is spun or cast into a thread or film. The thread or film will be colored a bluish black which is fast to light and comparatively fast to an alkaline scouring boil-off operation.

#### Example IV

A dye solution of Pontacyl Fast Red AS (Color Index No. 176) is prepared by dissolving the same in water to a concentration of about 2 grams per liter. An aliquot portion of the dye solution is added to a 23% solution of cellulose acetate in the proportion of about 8 cc. of the dye solution to 1000 grams of acetate solution, and the components suitably homogenized. Thread or film spun or cast from the resulting mixture is colored a reddish pink which is fast to light and comparatively fast to an alkaline scouring boil-off operation.

#### Example V

A dyed cellulose acetate solution, containing Pontacyl Light Yellow 3—G (Color Index No. 636), is prepared in accordance with Example I and spun or cast into a thread or film. The thread or film will be colored a light yellow which is fast to light and comparatively fast to an alkaline scouring boil-off operation.

#### Example VI

A dyed cellulose acetate solution, containing Pontacyl Fast Black BBO (Color Index No. 307), is prepared in accordance with Example III. The dyed cellulose acetate solution is spun or cast into a thread or film possessing a dark blue gray color which is fast to light and comparatively fast to an alkaline scouring boil-off operation.

Dyed threads and films produced in accordance with this invention are in most cases exceedingly fast to light and to the action of boiling water containing a small quantity of soap and sodium carbonate. This is a remarkably surprising result in view of the fact that those acid dyes which are water-soluble generally possess little or no affinity for cellulose acetate when applied to finished materials produced therefrom.

5 0 In general, dyes for cellulose acetate are expensive and do not exhaust well from dye baths; consequently, the dyeing of materials constructed of cellulose acetate, as practiced heretofore, is a comparatively expensive procedure.

5 5 The present invention makes possible the use of acid dyes, some of which are comparatively inexpensive, moreover, none of the dyestuff is lost in producing the colored materials.

A further advantage of the present invention 10 lies in the fact that the depth of color imparted to the material can be predetermined with great exactness by regulating the quantity of dye added to the cellulose acetate solution. Furthermore, any desired shade and color known is easily obtainable.

In contrast to the use of relatively complicated special colloidal mills and homogenization methods required in producing colored yarn by addition of insoluble colored pigments to the spinning 15 or casting solutions, the present invention requires no special mixing apparatus and only a short time to mix the dissolved dye uniformly into the acetate solution.

Since it is obvious that various changes and 20 modifications may be made in the above description without departing from the nature and spirit thereof, it is to be understood that the invention is not to be limited thereto except as set forth in the appended claims.

25 40 I claim:

1. The process of producing dull-colored artificial threads and pellicles composed essentially of a cellulose ester which comprises the steps of dissolving in a solvent therefor a water-soluble 25 acid dye which has substantially no affinity for said article when applied externally thereto from a dye bath and mixing said solution and a delustering agent with a solution of a cellulose ester, and forming said threads and pellicles from said 30 dyed, delustered ester solution.

2. The process of producing a dull-colored artificial thread composed essentially of cellulose acetate, which comprises the steps of dissolving in a solvent therefor a water-soluble acid dye which has substantially no affinity for said thread 35 when applied externally thereto from a dye bath and mixing said solution and a delustering agent with water, adding said mixture to a solution of cellulose acetate in acetone, and spinning said thread from the dyed, delustered acetate solu- 40 tion.

3. The process of producing artificial threads and pellicles composed essentially of an organic cellulose ester which comprises the steps of at least partially dissolving in a solvent therefor a 45 water soluble acid dye which has substantially no affinity for said threads and pellicles when applied externally thereto from a dye bath, mixing said dye solution with a solution of a cellulose ester, and forming said threads and pellicles 50 from the dyed ester solution.

4. The process of producing artificial threads and pellicles composed essentially of cellulose acetate which comprises the steps of at least partially dissolving in a solvent therefor a water soluble acid dye which has substantially no affinity for said threads and pellicles when applied externally thereto from a dye bath, mixing said dye solution with a solution of cellulose acetate 55 and forming said threads and pellicles from the 60 dyed acetate solution.

5. The process of producing dyed artificial threads and pellicles composed essentially of an organic cellulose ester which comprises the steps of dissolving in water a water soluble acid dye 65 which has substantially no affinity for said thread when applied externally thereto from a dye bath, mixing said aqueous dye solution with a solution of a cellulose ester, and spinning said thread from 70 said dyed ester solution.

6. The process of producing dyed artificial threads and pellicles composed essentially of cellulose acetate which comprises the steps of dissolving in water a water soluble acid dye which has substantially no affinity for said thread when applied externally thereto from a dye bath, mixing said aqueous dye solution with a solution of cellulose acetate in acetone and spinning said 75 thread from said dyed acetate solution.

FENTON H. SWEZENY. 80